

# UNITED STATES PATENT OFFICE.

LEON O. BRYAN AND WENDELL R. SWINT, OF WILMINGTON, DELAWARE, ASSIGNEES TO  
E. I. DU PONT DE NEMOURS & COMPANY, OF WILMINGTON, DELAWARE, A CORPORATION  
OF DELAWARE.

## EXPLOSIVE.

1,327,859.

Specification of Letters Patent. Patented Jan. 18, 1920.

No Drawing.

Application filed March 18, 1919. Serial No. 233,292.

To all whom it may concern:

Be it known that we, LEON O. BRYAN, of  
Wilmington, in the county of New Castle  
and State of Delaware, and WENDELL R.  
SWINT, of Wilmington, in the county of  
New Castle, and in the State of Delaware,  
have invented a certain new and useful improvement in Explosives, and do hereby declare that the following is a full, clear, and  
exact description thereof.

This invention relates to high explosives which are similar in their explosive properties to existing standard grades of dynamite.

The commercial explosives in which it  
has heretofore been proposed to incorporate  
trinitrotoluol may be said to fall in two  
main classes. In one class are compositions  
in which a small percentage of trinitrotoluol  
is used in conjunction with relatively large  
percentages of nitroglycerin for the purpose  
of producing the so-called low-freezing  
dynamite.

In explosive compositions of the other  
class, low percentages of trinitrotoluol are  
used with relatively high percentages of explosive salts having a high oxygen content such as ammonium nitrate, ammonium perchlorate, potassium chloride or perchlorate, or other oxidizing materials of this character. The purpose of the trinitrotoluol in this other class is to sensitize the ammonium nitrate or other explosive salt in order to make the composition capable of detonation with commercial blasting caps.

Explosives of the two types described above have certain advantages, but they also have certain disadvantages. Thus the low freezing dynamites are expensive to manufacture; they show a tendency toward exudation or leakiness of the liquid constituents; and users are liable to contract severe headaches by handling the explosive.

Explosives of the second class mentioned have three very serious disadvantages. Firstly, they are relatively insensitive to detonation. Secondly, they are very liable to become extremely hard after short periods of storage, in which hard condition they are very insensitive to detonation and are also very difficult to load into bore holes. Thirdly, they are usually very dusty and consequently dangerous, disagreeable, and unhygienic to manufacture.

The main object of our invention is to  
provide explosive compositions in which

these disadvantages are in a large measure avoided.

We have discovered that a very satisfactory explosive composition may be manufactured by combining as essential ingredients a relatively low percentage of nitroglycerin, a relatively high percentage of trinitrotoluol, and a relatively high percentage of sodium nitrate or other oxygen carrying salt, which, however, is not an explosive like ammonium nitrate, ammonium perchlorate, etc. One example of such an explosive would have the following composition:

|                |     |    |
|----------------|-----|----|
| Nitroglycerin  | 5%  | 70 |
| Trinitrotoluol | 40% |    |
| Sodium nitrate | 55% |    |

These ingredients may however be varied and other ingredients added in order to obtain certain desired characteristics, such as high or low strength, velocity, and density. For example, five typical formulas are shown below which are equivalent in strength to standard industrial dynamites as disclosed for example in Bureau of Mines' Bulletin No. 48, page 7.

| Per cent. strength | 25 | 30 | 35 | 40 | 50 | 85 |
|--------------------|----|----|----|----|----|----|
| Nitroglycerin      | 5  | 5  | 5  | 5  | 5  |    |
| Trinitrotoluol     | 15 | 25 | 25 | 25 | 35 |    |
| Sodium nitrate     | 55 | 57 | 57 | 57 | 43 |    |
| Wood pulp          | 2  | 3  | 3  | 3  | 3  |    |
| Corn meal          | 2  | 4  | 4  | 4  | 4  |    |
| Salter             | 2  | 4  | 4  | 4  | 4  |    |
| Chalk              | 1  | 1  | 1  | 1  | 1  | 90 |

It is understood that the percentages of these ingredients may be varied within certain limits, and other ingredients of similar characteristics substituted or added without departing from the scope of our invention. Thus we do not limit ourselves to the use of five per cent. (5%) nitroglycerin, since desirable results can be obtained from the use of from two to ten per cent. (2-10%) thereof.

The purpose of the nitroglycerin is to sensitize the explosive so that it will surely detonate with commercial blasting caps even under adverse conditions. It also acts to overcome the brittleness of explosives containing no liquid ingredients.

The trinitrotoluol is the most important constituent of the new composition and is used in various percentages depending upon

the strength which is desired. Although the trinitrotoluol used may be either the pure refined product or a low melting crude product, we have found the latter (melting at 65-70° C.) preferable because, on account of its somewhat oily nature, there is less tendency for the explosive to give trouble from dustiness during manufacture.

The function of the oxygen-carrying salt such as sodium nitrate is to furnish oxygen in the desired amount and to prevent the formation of noxious or deleterious fumes.

The combustible, non-explosive materials, such as wood pulp, corn meal, and sulfur, are added in some cases to impart the desired density, and also, especially when combined with sodium nitrate, to increase the strength of the explosive. In place of wood pulp and corn meal, we may use other carbohydrates as, for instance, flour. We do not limit ourselves to any particular percentage of combustible materials; it may be stated, however, that in some cases from five to seventeen per cent (5-17%) of such materials is preferred.

Explosives made in accordance with our invention as above described are thoroughly sensitive to detonation by commercial blasting caps, but at the same time are very insensitive to shock, fire, etc. They contain no liquid ingredient except the nitroglycerin and are consequently practically non-freezing. For the same reason they may be handled without the user suffering from the severe headaches caused by explosives containing large proportions of nitroglycerin. They are easily manufactured, the apparatus and equipment of the dynamite plant being suitable for the purpose. Within reasonable limits, any desired strength, velocity of detonation, and density may be obtained. They are comparatively free from dust which enables them to be handled during manufacture and use without the disagreeable and dangerous features attendant upon a dusty explosive. Finally, such explosives are cheaper to manufacture than the corresponding grades of ordinary dynamite.

We claim:

1. An explosive containing as the main explosive trinitrotoluol, nitroglycerin, and a non-explosive inorganic oxygen-carrying salt.
2. An explosive containing as the main explosive trinitrotoluol, from 2 to 10% of nitroglycerin, and a non-explosive inorganic oxygen-carrying salt.
3. An explosive containing as the main explosive trinitrotoluol which is present to the extent of at least 18%, nitroglycerin, and a non-explosive inorganic oxygen-carrying salt.

4. An explosive containing as the main explosive trinitrotoluol which is present to the extent of at least 18%, from 2 to 10% of nitroglycerin, and a non-explosive inorganic oxygen-carrying salt.

5. An explosive containing as the main explosive trinitrotoluol, nitroglycerin, and sodium nitrate.

6. An explosive containing as the main explosive trinitrotoluol, from 2 to 10% of nitroglycerin, and sodium nitrate.

7. An explosive containing as the main explosive trinitrotoluol which is present to the extent of at least 18%, nitroglycerin, and sodium nitrate.

8. An explosive containing as the main explosive trinitrotoluol which is present to the extent of at least 18%, from 2 to 10% of nitroglycerin, and sodium nitrate.

9. An explosive containing as the main explosive trinitrotoluol, nitroglycerin, sodium nitrate, and a combustible non-explosive material to impart the desired density to the composition and to increase its explosive strength.

10. An explosive containing as the main explosive trinitrotoluol, from 2 to 10% of nitroglycerin, sodium nitrate, and from about 5 to 17% of carbohydrate material.

11. An explosive containing from about 18 to 30% of trinitrotoluol, from about 60 to 40% of a non-explosive inorganic oxygen-containing salt, and from about 2 to 10% of nitroglycerin.

12. An explosive containing from about 18 to 30% of trinitrotoluol, from about 60 to 40% of a non-explosive inorganic oxygen-containing salt, from about 2 to 10% of nitroglycerin, and from about 17 to 5% of a non-explosive combustible material.

13. An explosive containing from about 30 to 50 parts of trinitrotoluol, from about 55 to 45 parts of an alkali-metal nitrate, and about 5 parts of nitroglycerin.

14. An explosive containing from about 30 to 50 parts of trinitrotoluol, from about 55 to 45 parts of an alkali-metal nitrate, about 5 parts of nitroglycerin, and not more than about 10 parts of carbohydrate material to impart the desired density to the composition and to increase its explosive strength.

15. An explosive containing about 30% of trinitrotoluol, about 54% of sodium nitrate, about 5% of nitroglycerin, an amount of wood pulp and corn meal totaling about 10%, and a small percentage of chalk.

In testimony that we claim the foregoing we have hereto set our hands.

LEON O. BRYAN.  
WENDELL R. SWINT.

Witness:

P. E. STRICKLAND.